# EUROPEAN PATENT APPLICATION

(11) **EP 4 379 101 A1**
(43) Date of publication of application: **05.06.2024**
(21) Application number: 22383142.1
(22) Date of filing: 29.11.2022
(51) Int. Cl.: D03D 15/283, D03D 15/50

(54) **A WOVEN FABRIC COMPRISING THERMOPLASTIC POLYMER FILAMENTS FROM NON-SHAPE MEMORY POLYMERS AND FILAMENTS FROM SHAPE MEMORY POLYMERS AND USES THEREOF**

(71) Applicant: Fundació Eurecat, 08290 Cerdanyola del Vallès (ES)
(72) Inventor: Jovancic, Petar, Sant Just Desvern (ES); Gonzalez Bertran, Judit, Barcelona (ES); Rodríguez Gutiérrez, Rosa, Barcelona (ES)
(74) Representative: Ponti & Partners, S.L.P

(57) **Abstract**

The present invention relates to a woven fabric comprising thermoplastic polymer filaments from a non-shape memory polymer **characterized in that** it further comprises up to 50% of filaments from a shape memory polymer with a glass transition temperature between 0 °C and 175 °C. The present invention also relates to the uses thereof.

## Description

### Field of the invention

The present invention relates to fabrics. In particular the present invention relates to woven fabrics comprising thermoplastic polymer filaments made from conventional non-shape memory polymers and stimuli sensitive polymers with shape memory effect triggered by temperature.

### Background

The knowledge of Shape Memory Polymers (SMPs), their commercial availability, the ways of use and integration into textile structures are in a very preliminary and unmethodical phase to be able to be offered to the market. A representative example is Shape Memory Polyurethane (SMPU). SMPU can be laminated, coated, filmed, foamed over textiles or even could be straight converted to continuous filament yarns using melt-spinning technology. When SMPU is laminated to a fabric, a smart fabric is formed. It is also possible to coat SM PU on a fabric such that its permeability changes as the wearer's environment and body temperature change to form an ideal combination of thermal insulation and vapour permeability for army clothing. Nevertheless, significant advances are still needed prior to putting these products into the market. Also, the subsequent textile application requires the generation of new knowledge on the way of production, mechanism of action and way of improving and adapting their properties according to specific needs and/or applications.

Woven fabrics containing thermoplastic polymer filaments (for instance PET) as already known in the prior art to have the problem that they have a low elastic deformation which after a prolonged use becomes irreversible (plastic deformation). Accordingly, there is the need to design a woven fabric having a higher (reversible) elastic deformation, in order to be adaptable to the user by changing its shape as a consequence of applied deformation and/or thermal stimulus.

The woven fabric as disclosed herein accomplishes the above mentioned goal. In addition, it has an additional advantage as regards of comfort/thermal properties, particularly water vapor resistance (Rₑₜ), thermal resistance (R_{ct}) and water vapor permeability index (iₘ) as these properties reversible change as well upon the deformation and/or applied thermal stimulus. Therefore, reversible elastic deformation originated from change from temporary to permanent shape of SMP filament yarns integrated into the woven fabric simultaneously results in significant change in comfort properties confirming that the woven fabrics disclosed herein is a sort of dynamic form structure responding to deformation and/or applied external temperature stimulus (dynamic reversible or thermodynamics textiles) as an exciting new generation of textiles that can detect, react and adapt to external conditions (deformation) or stimuli.

The innovative aspect of the technology discussed herein lies in the fact that a woven fabric with adjustable and reversible elastic deformation and thermodynamics properties can be designed by introduction of SMP filament yarns in a particular textile pattern, depending on the final application for which it is intended.

US7309104 relates to a seat assembly which includes a seat fabric, wherein at least a portion of the seat fabric comprises a yarn comprising a shape memory polymer adapted to undergo a change in a modulus of elasticity at a thermal transition temperature T_{g}. This document emphasizes only the elasticity of the fabric, but no reference is made to the reversible elastic deformation (shape adaptability) and thermodynamics' properties of woven fabric in contrast to fabric disclosed in this patent.

### Summary of the invention

In a first aspect, the present invention relates to a woven fabric comprising thermoplastic polymer filaments from a non-shape memory polymer **characterized in that** it further comprises up to 50% of filaments from a shape memory polymer with a glass transition temperature between 0 °C and 175 °C.

In a second aspect, the present invention relates to the use of the woven fabric according to the first aspect of the invention.

### Brief description of the drawings

Fig. 1 shows the different woven patterns for the shape memory filaments, wherein SMPU stands for Shape Memory Polyurethane and PES stands for polyester.
Fig. 2. Comparative recovery of sample 100% PES (100PES) and textiles with SMPU filaments by weft. Figure 2a shows the results of the water vapor resistance test (Rₑₜ).
Figure 2b shows the results of the thermal resistance test (R_{ct}). Figure 2c shows the calculations of the water vapor permeability index (iₘₜ).
Fig. 3. Scheme of the thermodynamic behavior in the thermal resistance test of a woven fabric with SMP filaments by weft and warp.
Fig. 4 shows an example of application in upholstery for seats (left: textile in PST; right: textile in TST).

### Detailed description of the invention

In a first aspect, the present invention relates to a woven fabric comprising thermoplastic polymer filaments from a non-shape memory polymer selected from polyester, polyamide, conventional polyurethane, conventional polylactic acid, polypropylene, polyethylene and mixtures thereof **characterized in that** it further comprises up to 50% of filaments from a shape memory polymer selected from polyurethane, polylactide-based polyurethane, polycaprolactone, polyether ether ketone and mixtures thereof with a glass transition temperature between 0 °C and 175 °C.

In the context of the present invention "woven fabric" and "textile" are used interchangeably in reference to the same concept.

The polyurethane and polylactic acid without SMP properties has been named as "conventional polyurethane" and "conventional polylactic acid", respectively.

SMP are segmented polymers having a microphase configuration. For example, in the case of polyurethane (SMPU), these segments are divided into hard segments (aromatic diisocyanates), which generate the permanent shape and are responsible for shape recovery; and soft segments (aliphatic polyethers or polyesters), which create the temporary shape and are responsible for shape fixity. The shape memory effect (SME) of these SMPUs is produced by the thermodynamic incompatibility between the hard and soft segments. Depending on the formulation, transitions may be located at the melting temperature (Tₘ) or the glass transition temperature (T_{g}) of the hard segment (Tₘₕ or T_{gh}, respectively), and at the Tₘ or T_{g} of the soft segment (Tₘₛ or T_{gs}, respectively). When stress is generated in the tensile direction, the deformation, in the form of the orientation of the polymer chains, is stored elastically in the soft segment, while the hard segment remains virtually unchanged. In order to obtain the effective functionality of the SMPU, attractions between the polymer chains of the hard segments must be maintained in the presence of stress, while the soft segment absorbs said stress and lengthens its chains.

The same can be applied to polylactide-based (PLA-based) polyurethane (PLAU) with SMP properties. In this particular case, the hard segments would be PLA diol isophorone diisocyanate (IPDI) and the soft segments would be different diisocyanates. In particular reference is made to Wang, W., Ping, P., Chen, X., & Jing, X. (2007). Shape memory effect of poly (L-lactide)-based polyurethanes with different hard segments. Polymer international, 56(7), 840-846, where a further explanation about PLA-based polyurethanes with SMP properties is provided.

In contrast with the prior art, the fabric according to the present invention has an improved elasticity of the thermoplastic polymer filaments with a reversible deformation.

In a preferred embodiment, the non-shape memory polymer is polyester.

In another preferred embodiment, the shape memory polymer is polyurethane with a glass transition temperature between 0 °C and 100 °C.

In a further preferred embodiment, the non-shape memory polymer is polyester and the shape memory polymer is polyurethane with a glass transition temperature between 0 °C and 100 °C.

The unique capability to deform in predefined conditions (temporary shape, TS) and recover back to its original shape (also called permanent shape, PS) upon being triggered by different external stimuli such as heat, radiation, pH, hydration, mechanical, magnetic, and electrical influences, etc. make polyurethanes (PUs) a versatile material with extraordinary characteristics (high recoverable strain up to 400%). The intrinsic shape memory ability of the PUs (shape memory PUs - SMPUs) is due to the presence of macro domains of soft and hard segments in its bulk. The presence of hard segment provides the mechanical strength which is responsible for it to remember the initial shape after deformation whereas the energy for dissipation is stored by soft segments providing the desired force to PU to revert it to its initial form by the action of external stimuli. SMPU is a class of polyurethane that is different from conventional polyurethane in that these have a segmented structure and a wide range of glass transition temperature (Tg). A large, reversible change in the elastic modulus across the Tg is what makes the shape change and shape retention possible. Conventional PUs cannot completely restore their residual inelastic deformation upon heating. In contrast, SMPUs can recover all the residual plastic deformation up to 400% through a micro-Brownian movement triggered by heating them above their glass transition temperature (Tg).

The conventional polyurethane (e.g., from 1, 6-hexane diisocyanate and 1,4-butane diol) is composed of diisocyanate and either short chain glycol or long chain polyethers or polyester glycol having multiple hydrogen bonding between - NH- and -OC- groups, which result in high hardness and strength and low degree of solubility. Also, conventional PU could be obtained by reaction of long chain, non-crystalline, unbranched, OH-functional polyethers or polyesters (which do not contain free or low molecular weight glycols) with stoichiometric amounts of diisocyanates containing about 4 to 7% urethane groups. The intermolecular forces for polyethers and polyesters PU are weak van der Waals forces. As a result, hardness and strength are comparatively low and the product exhibits rubber-like properties. Both types of PU products have only one phase and are used for the obtention of cross-linked hard products (PU rigid foams, non-textile coatings etc.).

Nevertheless, SMPUs are composed of: a) long chain polyether or polyester polyol, b) diisocyanate (aromatic diisocyanates are most commonly used for SMPU) and c) glycol or diamine (chain extender). Diisocyanate and chain extender are hard segments, on the other hand long chain polyol is soft segment. These types of polyurethane are characterized by a segmented structure (block copolymer structure) and the morphology depends on chemical composition and the length of the segment (block). The hard blocks are formed by the reaction of diisocyanate with low molecular weight glycol, or diamine (chain extender) whereas the soft segments are formed by polyol (oligomer). The hard blocks constitute about 30-50% by weight of the total polymer. The microphase separation of these two dissimilar blocks due to its thermodynamic incompatibility produces regions of hard blocks concentration (domains) which act as cross-link points for the soft blocks. Hard segments can bind themselves via hydrogen bonding and crystallization, making the PU very solid below melting temperature. The segmented network structure can be easily deformed above glass transition temperature (Tg) to give a temporary shape, the original shape can be recovered when the material heat above the glass transition temperature. The shape memory effect can be controlled via molecular weight of soft segment, mole ratio between hard and soft segment, and polymerization process of PU.

In a typical shape memory cycle of thermally induced SMPUs, the sample is firstly heated freely, deformed from its original permanent shape to a temporary shape, and then cooled down. The sample can maintain the temporary shape and is also able to spontaneously recover to the permanent shape once being heated. Such a capability is also known as one-way shape memory effects (SMEs), since the sample cannot recover to the temporary shape unless being deformed manually. Polymers of one-way SMEs (or one-way SMPs) are thus suitable for applications where only a single temporary-permanent shape recovery cycle is demanded such as self-deploying biomedical devices or SMPU-based textile fabric that is scope of this patent.

However, reversibility of the shape shifting is necessary for some applications like soft actuators, sensors, actuated porous membranes or artificial muscles, where the use of two-way shape memory polymers (2W-SMPs) capable to remember two different shapes, both a low and a high temperature shape, even without external force is recommended. There exist four kinds of 2W-SMPs classified by the molecular strategies towards their preparation: liquid crystalline elastomers (LCEs), semi-crystalline networks (SCNs), two-way shape memory composites or laminates (2 W-SMC) and interpenetrating polymer of elastomeric and crystalline networks (IPNs). However, the cyclic behavior of 2W-SMPs is not yet as well understood as that of the one-way-effect. The cyclic use of the one-way-effect with external reset force is, in many cases, a more economical solution than 2W-SMPs. Some SMPUs or its composites are even triple, or quadruple based on the number of glass transition temperatures and soft and hard contents are described [See Taylor Ware; Keith Hearon; Alexander Lonnecker; Karen L. Wooley; Duncan J. Maitland; Walter Voit; Triple-Shape Memory Polymers Based on Self-Complementary Hydrogen Bonding. Macromolecules 2012, 45, 1062-1069, 10.1021/ma202098s; and Jiayu Xian; Jieting Geng; Yan Wang; Lin Xia; Quadruple-shape-memory effect of TPI/LDPE/HDPE composites. Polymers for Advanced Technologies 2017, 29, 982-988, 10.1002/pat.4209]. Transition temperature (T_{g}), shape fixity (R_{f}), shape recovery ratio (Rᵣ), maximum recoverable strain (εₘₐₓ), and maximum recovery stress (σₘₐₓ) are the important parameters that are used to describe shape memory effects of a polymeric material.

The micro morphology of SMPU strongly affects its mechanical properties and consequently the SME. There are many factors, which can influence this morphology SMPUs: chemical structure, composition, and sequence-length distribution of the hard segments, overall molecular weight and its distribution as well as the SMPU processing parameters, such as thermal conditions and applied mechanical forces applied during the melt-spinning process used for obtaining of SMPU filaments.

In a further preferred embodiment, the shape memory filaments are monofilaments, multifilaments or a combination thereof.

Regarding the type of weaving, in a preferred embodiment, the shape memory filaments are weft filaments, warp filaments or a mixture thereof.

Furthermore, in another preferred embodiment, the shape memory filaments have a type of woven pattern selected from plain, twill, satin and a combination thereof. Figure 1 shows the different distribution of an example of the present invention, wherein PES is the non-shape memory polymer and SMPU is the shape memory polymer.

If a twill woven pattern is chosen, this in turn can be selected from Right Hand Twill, Left Hand Twill, and Broken Twill and a combination thereof.

If a plain woven pattern is chosen, this in turn can be selected from Rib Weave, Matt Weave, Basket Weave and a combination thereof.

The woven fabric of the present invention, including any of the embodiments disclosed above or any combination thereof, comprises up to 50% of filaments from a shape memory polymer. These filaments may further contain an additive selected from the group consisting of carbon black, carbon nanotubes, graphene, vapor-grown carbon fiber, carbon nanofiller, attapulgite, sepiolite, bentonite, glass fiber, silver, cloisite 10A/cloisite 30B, carbon nanorod, nanopaper, cellulose nanofiber and a mixture thereof.

These additives allows the filaments to have:
- an optimal or modulated recovery;
- an increased tensile strength;
- a higher electrical conductivity; and
- a different glass transition temperature which could be useful depending on the intended application.

It is well known in the art that SMP properties are influenced by the presence of additives and that, depending on their distribution in the matrix, as well as their nature, morphology and content, they may have distinct effects. See Meng, Q., & Hu, J. (2009). A review of shape memory polymer composites and blends. Composites Part A: Applied Science and Manufacturing, 40(11), 1661-1672.

In a preferred embodiment, said additive is selected from the group consisting of carbon black, carbon nanotubes and a mixture thereof.

Regarding the amount of the additive in the filaments from a shape memory polymer, in a preferred embodiment, it is lower than 7 wt %.

In a further preferred embodiment, the amount of the additive in the filaments from a shape memory polymer is lower than 3 wt %.

In a second aspect, the woven fabric of the present invention, including any of the embodiments according to the first aspect or any combination thereof, is used in upholstery. In particular, this upholstery is for a vehicle seat or for home furniture.

In another embodiment, the woven fabric of the present invention, including any of the embodiments according to the first aspect or any combination thereof, is used in home textiles. In particular, these textiles are bed linen, mattress, cushions.

In another embodiment, the woven fabric of the present invention, including any of the embodiments according to the first aspect or any combination thereof, is used in a medical applications/biomedical textile. In particular, these textiles are bandages, dressings, patches, etc.

These potential applications have in common a fabric that dynamically adapts, both in shape and in thermal comfort, to the needs of a user.

Figure 4 shows an example of application in seat upholstery. Traditionally, woven fabrics are used for seat upholstery, since they must meet specific safety design standards, as well as optimal thermal comfort parameters. Upholstery fabrics must also meet certain requirements, even more demanding when used in motor vehicles. These requirements may include high abrasion resistance, resistance to UV degradation, tensile strength, pilling, flammability, and seam strength. Polyester fibers meet these demands at a relatively low price, in addition to low water absorption, excellent flexibility and wrinkle resistance. The problem is that the upholstery process is carried out with high tensions, so the textile has very little deformation and this does not allow the textile to adapt to the body. The incorporation of SMP filaments would allow this adaptability through the deformation of the SMPU filament.

As for the process for obtaining the woven fabric as claimed herein, it could be noted that woven fabrics are produced on industrial or semi-industrial looms and are made up of interweaving yarns in the warp direction and yarns in the weft direction. The warp yarns are located parallel in the longitudinal direction of the fabric. They are the base on which the passes of the weft yarns intersect in the transverse direction. The process requires minimal tension in both directions so as not to interfere with interweaving. The different variants of fabrics based on plain, twill, satin and their combinations will depend on the type of interweaving that is made of the weft and the warp.

As for the specific SMP introduction process, the filaments in temporary shape will be introduced into the woven fabric. The force and strain for the incorporation of the SMP filaments by weft and warp will be the minimum necessary to allow the weaving process, since the filaments show a low resistance to deformation compared to other thermoplastic filaments/fibers without shape memory.

The invention will be now illustrated by way of one or more examples which do not intend to limit the scope of the invention.

### Examples

### Example 1. Production of the woven fabric of the invention

The polymer used was a SMPU, ether-based polyurethane (MM4520 and MM6520 grade) having a Tg of 45°C and 65°C respectively, provided by SMP Technologies Inc. Japan. Pure SMPU pellets were melt-spun with a Collin Tech-Line extruder followed by a first drawing zone (stretching roller A), a hot-air stretching furnace and a second drawing zone (stretching roller B). A 0.6 mm diameter nozzle was used to obtain filaments with an adequate diameter for multi-sectorial applications. Temperature ranges and other parameters of the extrusion process were adjusted to the viscosity of the SMPU pellets (8.4 g/10min). Textured PES yarns, kindly supplied by Antex (Spain), were used for the warp (450 dtex) and for the weft (300 dtex).

Plain (P), twill 2.2 (T2) and twill combination (TC) weave fabrics were produced on a Studio 5020 narrow laboratory loom (Techn inc, Taiwan). The tension used in the warp and the speed of the rapier were adjusted to allow the introduction of SMPU filaments in woven textile. SMPU filaments were incorporated in the temporary shape to generate thermodynamism in textiles. The same warp and weft density was used for all the fabrics. PES yarns were used in both warp and weft and SMPU filaments were introduced only per weft (OW) or per weft and warp (WW) at different ratios: 3PES:1SMPU (25SMPU) and 1PES:1SMPU (50SMPU). For comparative purposes, weave fabric 100% PES (1PES) were also produced. Table 1 shows a summary of the composition and nomenclature used.

### Example 2

The tensions generated in the production process of the fabric and the subsequent heat treatment to return to permanent shape (PSF) reduced the length of the SMPU filament embedded in the textile. The heat treatment was performed without applying any external force using a STUART Digital Hotplate SD 500.

The dimensional (width) changes of fabrics directly after the weaving process (relaxation shrinkage) and when they are subjected to heating up over Tg were also measured and referred to as TSF (temporary shape of the fabric) and PSF (permanent shape of the fabric). Five measurements were taken along the fabric in weft direction (TSF and PSF).

Table 2 shows the relaxation shrinkage values of the weft fabric after the weaving process, in the temporary shape of textile TSF, and after weaving and subjected to heat treatment, in the PSF, relative to the fabric during the weaving process. It also shows the textile recovery produced by the heat treatment.

Textiles with SMPU filament yarns presented higher shrinkage than the 100PES sample in both TSF and PSF. However, the increase in weft shrinkage is more significant in the case of PSF due to the effect of heat treatment over the Tg on SMPU filament yarn/fabrics characteristics. Due to significant elastic recovery of SMPU filament yarns over the Tg, the residual shrinkage is ruled by their content. The higher SMPU filaments yarn content is, the higher residual shrinkage is obtained. It was observed that shrinkage in weft increased when integrating the filament by warp and weft as well as when using twill woven pattern (TC and T2).

These results show us that the shrinkage capacity of the SMPU filament yarn is affected by the type of fabric used, twill affects it to a lesser extent than plain. It is also affected by the direction in which it is inserted, since by warp and weft the shrinkage occurs in both directions, offering less resistance.

### Example 3.

The thermal comfort of all the textiles in the TSF and in the PSF was analyzed to know the dynamism of each textile in the face of an increase in temperature. Thermal comfort is determined by the thermal permeability index (iₘₜ), and to determine it, it is necessary to analyze water vapor resistance (Rₑₜ) and thermal resistance (R_{ct}) of the fabrics. According to Verdu P, Rego JM, Nieto J, et al. Comfort Analysis of Woven Cotton/Polyester Fabrics Modified with a New Elastic Fiber, Part 1 Preliminary Analysis of Comfort and Mechanical Properties. Text Res J 2009; 79: 14-23, textiles with vapor permeability index values below 0.3 can be considered thermally comfortable to be used as garments.

### Example 4

The water vapor resistance (Rₑₜ) and thermal resistance (R_{ct}) of the fabrics were determined using a Permetest skin model instrument by Czech Sensor company. The relationship between both parameters, Rₑₜ and R_{ct}, gives the water vapor permeability index (iₘₜ) and indicates the degree of thermal comfort. Figure 2 illustrates the increase in each of the thermal parameters analyzed (Rₑₜ, R_{ct} and iₘₜ) of textiles with SMPU filament yarns and the 100PES samples in TSF and PSF.

Figure 2a shows the results of the water vapor resistance test (Rₑₜ) and figure 2b the results of the thermal resistance test (R_{ct}). The results indicated that in all cases the textiles with SMPU filament yarns showed higher values than the textiles with 100% PES. These values increased with the content of SMPU filament yarns in weft and when incorporating SMPU filament yarns by warp. In the Rₑₜ, similar values were observed between the different textile structures in the TSF, while the values were higher in the twill structures in the PSF. In the R_{ct} the values were clearly higher in the twill structures both in the TSF and in the PSF, especially in the twill 2.2 in the PSF.

Figure 2c shows the calculations of the water vapor permeability index (iₘₜ). The results indicated an increase in the values of the textiles that incorporate the SMPU filament yarns. It is worth noting the decrease observed in the sample 25SMPUWW-P with respect to the samples of plain fabrics that incorporate SMPU filament yarns only per weft. This is due to a greater increase of the Rₑₜ with respect to the R_{ct} compared to the other plain textiles with SMPU filament yarns. On the other hand, it is worth mentioning the clear increase in iₘₜ in the 25SMPUWW-T2 sample in the PSF that reached the limit value considered thermally comfortable due to the high value obtained in the R_{ct} in proportion to the lower increase in Rₑₜ.

This comparison shows that a clear thermodynamic regulation is possible with a low impact on the thermal permeability index, so it remains thermally comfortable.

A fabric woven with integrated SMPU filaments for weft and warp improves the dynamic thermal comfort obtained with textiles with SMPU filaments only in weft, by recovering the permanent shape in both directions of the textile.

Figure 3 illustrates the dynamism of the textile with SMP filaments by weft that, in the face of an increase of environment temperature, produces an increase in thickness and density in the textile in the TSF (textile in the PSF), thereby regulating the transmission of environment heat.

### Example 5

The mechanical resistance of the textiles was analyzed to understand how the incorporation of the SMPU filament yarn affects the deformation of the textile. Fabrics are only analyzed in the PSF because they are the ones that show the full force/strain curve that the TSF is a part of.

The tensile tests were conducted according to UNE-EN ISO 13934-1: 2013 standard using a static testing Zwick / Roell machine. Five specimens in the PSF of 50mm wide and 100mm length were prepared for each fabric. Any preload was applied and the testing speed was set to 100mm/min. Table 3 shows the results of the initial zone of the force-deformation curve where the change in stress is obtained due to the beginning of the resistance of the PES fiber. This change is indicated as the point of connection Fᵣ and εᵣ.

It was observed that both parameters F₁ and ε₁, increased with increasing proportion of SMPU filament yarn. This increase in F₁ was clearly higher in the samples with SMPU filament yarns by weft and warp (WW) than those obtained with SMPU filament yarns only by weft (OW). This phenomenon may be due to the higher concentration of SMPU filament yarns per cm. In ε1, this increase was also observed, the same as in the case of F1, except for the 25SMPUWW-P sample, which obtained a value higher than the 25SMPUOW-P sample but lower than the 50SMPUOW-P sample. This could be due to the influence of the SMPU filament yarns that are part of the warp that, on the one hand, allow the increase with respect to the 25SMPUOW-P textile but continue to limit the deformation due to the interlacing of the structure.

In this test, the limit force that allowed an elastic or recoverable deformation was obtained for all fabrics with SMPU filament yarn that was used in the tensile tests of the shape memory effect (SME).

### Example 6

The shape memory behaviour (normally called shape memory effect) of textiles is analyzed to understand the temporary shape fixing and permanent shape recovery capabilities of all textiles.

To determine the shape memory effect, the temporary shape fixation (fixity ratio, R_{f}), and the recovery to permanent shape (recovery ratio, Rᵣ) different tests were performed using a Zwick/Roell dynamometer test machine. Two types of tests were carried out: a first test applying a limit recovery tensile force of the textile memory (F₁) of 25N, obtained in the force-deformation test, at 80°C. This test was carried out in the direction of the weft with the textiles with SM PU filament yarns per weft and the 100PES-P sample and the values were obtained from the average of 3 tests. The dimensions of the specimens were 50x100 mm.

A second test applied a bending force of limit recovery of the memory of the textile of 1N at 80°C. This test was carried out with the different PES textiles and with the textiles with SMPU filament yarns in weft and warp, obtaining the mean values of 2 tests. The dimensions of the specimens were 220x220mm. These specimens were held at all ends on a holding structure that maintained tension for all samples. Table 4 shows the results of the shape memory effect (SME) tests that are determined by the fixation ratio (R_{f}) and recovery ratio (Rᵣ).

In the test of the shape memory effect by tensile force, the textiles with SMPU filament yarns show higher values of the fixation ratio (R_{f}) and the recovery ratio (Rᵣ) with respect to textiles with 100% PES which show lower values, especially in R_{f}.

In the flexural force shape memory effect test, textiles with SMPU filament yarns showed higher values of R_{f} compared to textiles with 100% PES, however they showed similar values in Rᵣ.

## Claims

1. A woven fabric comprising thermoplastic polymer filaments from a non-shape memory polymer selected from polyester, polyamide, conventional polyurethane, conventional polylactic acid, polypropylene, polyethylene and mixtures thereof **characterized in that** it further comprises up to 50% of filaments from a shape memory polymer selected from polyurethane, polylactide-based polyurethane, polycaprolactone, polyether ether ketone and mixtures thereof with a glass transition temperature between 0 °C and 175 °C.

2. The woven fabric of claim 1, wherein the non-shape memory polymer is polyester.

3. The woven fabric of claim 1 or 2, **characterized in that** said shape memory polymer is polyurethane with a glass transition temperature between 0 °C and 100 °C.

4. The woven fabric of any of claims 1 to 3, **characterized in that** said shape memory filaments are monofilaments, multifilaments or a combination thereof.

5. The woven fabric of any of claims 1 to 4, **characterized in that** the shape memory filaments are weft filaments, warp filaments or a mixture thereof.

6. The woven fabric of any of claims 1 to 5, **characterized in that** the shape memory filaments have a type of woven pattern selected from plain, twill, satin and a combination thereof.

7. The woven fabric of claim 6, **characterized in that** the twill woven pattern is selected from Right Hand Twill, Left Hand Twill, and Broken Twill and a combination thereof.

8. The woven fabric of claim 6, **characterized in that** the plain woven pattern is selected from Rib Weave, Matt Weave, Basket Weave and a combination thereof.

9. The woven fabric of any of claims 1 to 8, further comprising an additive selected from the group consisting of carbon black, carbon nanotubes, graphene, vapor-grown carbon fiber, carbon nanofiller, attapulgite, sepiolite, bentonite, glass fiber, silver, cloisite 10A/cloisite 30B, carbon nanorod, nanopaper, cellulose nanofiber and a mixture thereof.

10. The woven fabric of claim 9, **characterized in that** the additive is selected from the group consisting of carbon black, carbon nanotubes and a mixture thereof.

11. The woven fabric of claim 9 or 10, **characterized in that** the additive is present in the filaments from the shape memory polymer in a percentage lower than 7 wt %.

12. Use of the woven fabric of any of claims 1 to 11, in upholstery.

13. Use of the woven fabric of claim 12, **characterized in that** the upholstery is for a vehicle seat or for home furniture.

14. Use of the woven fabric of any of claims 1 to 11, in home textiles.

15. Use of the woven fabric of any of claims 1 to 11, in medical applications or biomedical textile.
